

May 22, 1934.

J. H. LUCAS

1,959,376

PROCESS FOR PRODUCING METAL POWDERS

Filed Sept. 26, 1930



INVENTOR  
James H. Lucas  
BY  
Ward, Cady & Neal  
ATTORNEYS

## UNITED STATES PATENT OFFICE

1,959,376

## PROCESS FOR PRODUCING METAL POWDERS

James H. Lucas, Elmhurst, N. Y., assignor to  
Nichols Copper Company, New York, N. Y., a  
corporation of New York

Application September 26, 1930, Serial No. 484,540

13 Claims. (Cl. 204—1)

This invention relates to a process and apparatus for producing metal powders.

A method and apparatus used heretofore for this purpose included spaced cathode rods and anodes dipping into an electrolyte bath adjacent said rods. The bath was an electrolyte of copper sulphate and sulphuric acid. Current passing through the electrolyte from the anodes to the cathode rods deposited copper on these rods in a fluffy mass or slime. The deposit on the rods was allowed to build up for about 15 minutes and at 15 minute intervals the rods where given a jarring by hand which caused at least some of the deposit to fall off and into the bottom of the electrolyte bath from which it was ultimately removed, and after washing and drying was screened to secure a copper powder of the desired particle size.

This old system presented disadvantages which may be briefly summarized as follows:—The building up of the copper deposit on the rods caused the rods to increase in size, thus changing the density of the current at the cathode. The density of current determines the particle size of the copper deposit on the rods and if the density changes as is the case where the deposit on the rods is constantly changing, the size of these particles varies. When the particles, therefore, were jarred off of the rods, particles of varied size were recovered from the bottom of the electrolyte bath. The variation in density of the current caused some large crystals to form along with those of a smaller size, thus necessitating sieving to remove the large crystals. According to the old system where it was desired to obtain crystals which would pass through a 200 mesh or better, with the jarring of the rods every 15 minutes it was found that about 20% of the total copper powder produced consisted of crystals too large to pass through the 200 mesh sieve. In addition it was necessary to use substantially pure copper anodes due to the fact that any impurity separated from the anodes during the course of deposition would fall into the bottom of the electrolyte bath and become mixed with the copper powder jarred from the rods where a substantially pure copper powder was desired. It was, therefore, necessary to start off with anodes of relatively high purity in order to avoid the presence of these impurities in the resulting copper powder, such as iron, silver, tin, lead and zinc. In addition in the old system the rods required replacing about once a week due to the fact that at the point where the rods entered the electrolyte, oxidation by the old system occurred with

eating away of the rods at that point until they were finally eaten through and dropped to the bottom of the tank.

An object of the present invention accordingly is to do away with these difficulties and to provide a simple efficient apparatus and process for producing metal powders such as copper powder which shall be simple, relatively inexpensive to operate, requiring little supervision, doing away with the necessity for renewal of parts as in the old system. Other objects will be in part obvious and in part pointed out hereinafter.

The invention accordingly comprises the novel apparatus and combinations thereof, as well as the novel processes and steps of processes which may be carried out in such apparatus, specific embodiments of which are described herein by way of example only and in accordance with the manner in which I now prefer to practice the invention.

In the accompanying drawing wherein I have shown a preferred embodiment of my apparatus, Fig. 1 shows a somewhat diagrammatic side elevation, partly in section, of an apparatus embodying my invention. Fig. 2 is a plan view corresponding to Fig. 1 and showing the relative positions of anodes and cathodes. Fig. 3 is a detailed view of the spray used for washing away the copper powder scraped off the cathodes, and Fig. 4 is a somewhat enlarged detailed view of a device for controlling the overflow of electrolyte from the electrolyte bath.

Referring now to this drawing, I shall describe the apparatus as applied to the production of copper powder of a desired degree of purity and containing a copper content which may be as high as 99.75%. It is to be understood, however, that the invention herein is not restricted to apparatus or method of producing copper powder but is applicable generally to production of other metallic powders which are susceptible to electro-deposition in powder form.

The numeral 1 designates a series of spaced copper supports supporting in turn copper anode plates 2 here shown as in the form of approximately 90° segments. The plates 2 may be made of relatively impure copper. It is not necessary that these plates be made up of copper of a high degree of purity as was the case with the anode plates used in the prior operation described above. Of course if desired such pure copper plates may be used, but their employment is not important. Thus a considerable saving in anode expense may be effected. These anode plates are suitably supported on the bars 1 by means of wires 3

passing through holes in the plate. The bars 1 are in turn supported by the sides of a lead-lined wooden tank 4 provided with a dished bottom leading to a valved exit which will be described 5 later.

The tank 4 contains an electrolyte bath of copper sulphate and sulphuric acid.

The cathodes consist of a series of rotating copper disks alternating with the anodes 5 and 10 submerged edgewise in the electrolyte bath.

In order to provide the proper current density passing between the anodes and cathodes, a device which will be described later is provided to control the overflow of the electrolyte and hence 15 its depth. The depth of immersion of the electrodes in the electrolyte determines the current density. For producing a commercial copper powder with this apparatus, I prefer to submerge the cathodes to about one-quarter their depth.

20 The cathodes are mounted on a shaft 6 supported in bearings 7 at either end of the tank 4, the bearings being suitably insulated from said tank. Mounted on this shaft is a steel sprocket 8 driven by a chain 9 from a smaller sprocket 10 25 mounted on its shaft 11 supported on said tank. The sprocket 8 is suitably insulated from the shaft 6 by means of an insulated bushing.

A source of current supply, not shown, has its 30 positive pole connected to the anodes through wiring 12 attached to a conducting strip 13 with which the anode bars 1 are in contact. The negative pole is connected by means of wires 14 connected to the bearing block 7.

When current passes the anodes to the rotating 35 cathodes, a thin fluffy deposit or slime of copper is deposited on that portion of the cathode disk 5 which is submerged. The rotation of these disks is preferably continuous and therefore there is a continuous deposition of copper 40 made on both faces thereof. It will be noted that the disks 5 are rotating in clockwise direction as shown in Fig. 1 and therefore the copper is being deposited from the moment that the disk enters the electrolyte on the right side of 45 the tank until it emerges from the left side, then from the left side the copper remains on the disk until it comes to a position just in advance of where it enters the tank. At this point a scraping device is provided shown more clearly in 50 Figs. 1 and 3. The scraping device consists of two troughs 15, the inner edges of which are sharpened to form scrapers 16 and contact each with the near face of one of the cathode disks. These pairs of scrapers are provided for each 55 of the cathode disks in the series. Immediately above each of the troughs 15 are positioned sprays 17 which are connected in a system to be later described for spraying electrolyte on to the copper as it is scraped off. The stream of electrolyte 60 thus carries along the particles of copper with it and the troughs being inclined towards a series of exit pipes 18. The electrolyte with the copper passes through these pipes and into a settling tank 19.

65 The sprays as noted are part of a circulating system. This circulating system supplies electrolyte for washing and conveying away the copper scraped from the cathodes as noted and includes heating devices for maintaining the electrolyte bath in the tank 4 at about 120° F. which 70 is the preferred temperature for depositing the copper in proper size under the preferred conditions. This system not only includes the sprays 17, pipes 18 and settling tank 19, but also has a receiving tank 20, a heating tank 21 and a pump 75

22. The electrolyte bath, the tanks 19, 20, 21 and pump 22 are all connected by piping, so as to permit a continuous flow of electrolyte heated to 120° F. or a selected temperature as desired.

The tank 4 is connected by means of an L shaped pipe 22a with a pipe 23 leading to an overflow box 24 for the tank 19 which communicates by pipe 25 with receiving tank 20. Situated in the L pipe is a short length of pipe 26 so designed that it projects into the upright portion of the L to give an exit for electrolyte from the tank 4 at the desired height to give a proper current density between the anodes 2 and cathodes 5. If the pipe 26 reaches nearly to the top of the tank 4, the exit through this pipe 26 will insure that the electrolyte bath in tank 4 will rise until it overflows 26 and the depth of liquid then in the tank 4 will be equal to the distance between the bottom of the tank and the top of the pipe 26. By substituting a medium length of pipe somewhat shorter than the one just mentioned, a slightly lower depth of liquid may be maintained and this depth may be varied as desired within the limits of the height of the upright member in the L, by changing the lengths of the pipe 26. Of course the L may have the height of the upright member varied as required.

The receiving tank 19 receives the electrolyte with copper particles suspended therein and when conveyed to this receiving tank, the particles settle out therein, the electrolyte passing off through a pipe 27 into the overflow box 24 and then through the pipe 25 to the receiving tank 20. The pump 22 is connected directly to the receiving tank. It is preferably a motor driven centrifugal pump and is connected by means of piping 28 to deliver into the upper portion of heating tank 21. In this heating tank is a series of steam coils 29 connected with a source of steam and to a discharge not shown. The electrolyte in this tank 115 is heated indirectly by the steam and when heated to approximately 120° F. or other desired temperature passes out through the valved pipe 30 into a pipe 31 which is branched, one branch supplying electrolyte to the sprays 17 and the other 120 branch 32 delivering the heated electrolyte to the tank 4.

The settling tank 19 is provided with a valve 33 at an exit in the bottom thereof, the valve being manually operable by a valve stem 34. When the 125 valve 33 is pulled up, the copper particles with electrolyte pass through a pipe 35 into a delivery pipe 36 from whence it passes into a wheeled filtering car 37 where it is received on a filter tray 38, the electrolyte being sucked off through 130 the suction filter of the car and being later washed by water, care being taken to insure that the copper particles are maintained under the electrolyte or covered with water during the process of removal of the electrolyte, and up to 135 the time the tray 38 is withdrawn and placed in the vacuum dryer. This part of the operation is preferably like that described in the application of Eugene Fitzpatrick, et al. Ser. No. 287,033 filed June 20, 1928.

As noted above the anode plates may be of impure copper and where this is the case it will be obvious that impurities therein, which are not deposited by electro-deposition, will fall to the bottom of tank 4 collecting on the dished surface 145 thereof. In the center of the bottom is a valve 39 seated in an L projection of the pipe 36 provided with a valve stem 40 which may be operated from below to unseat the valve upwardly to allow the impurities in the tank 4 to run out 150

through the pipe 36. These impurities will collect at a rate depending on the purity of the anodes. Tank 4 is cleaned out as often as is necessary and of course these impurities are kept 5 separate from the copper received in the pipe 36 from the settling tank 19. The impurities are not only handled separately in this pipe but they are preferably handled separately in the filter car and in the subsequent drying process.

10 In carrying out the process of my invention, I prefer to proceed as follows in producing a copper powder. Current is passed from the anodes 2 to the rotating cathode copper disks. Under preferred circumstances the current density at 15 the anodes will average approximately 85 amperes per square foot while the current density at the cathodes will average approximately 250 amperage per square foot. I rotate the copper disks at the rate of about one or less revolutions per minute, the cathodes being submerged to about one-quarter of their depth in the electrolyte to give the desired current density. The anode is immersed substantially entirely. I regulate the current density to the preferred amount for 20 the size of copper particles desired by selecting a pipe 26 of the proper height so that the level of the electrolyte in the tank 4 is sufficient to give the current density desired. The preferred electrolyte contains from about 2.3% to 2.45% of copper, as copper sulphate, and from about 11.3% to 11.4% sulphuric acid. The copper deposited, as the rotating cathodes pass through the tank 4, then passes around through an angle of somewhat less than 180° until it reaches the trough 25 15 with its scraper where the deposit is scraped off and washed away by electrolyte flowing through the spray 17, from the tank 21. I prefer to maintain the electrolyte at 120° F. and for this purpose a circulating and heating system is provided. The electrolyte flowing from the tank 4 passes downwardly through the overflow box 24 of the settling tank and thence it passes into the receiving tank. The copper particles washed away by the spray 17 flow into the pipes 18 and 30 thence into the settling tank where the copper settles out and may be removed when collected in sufficient quantity from the settling tank 19. The excess electrolyte passes into the settling tank overflow box and then into the receiving tank 20. From the latter the pump 22 pumps the electrolyte up to the heating tanks 21 where it is heated and then allowed to flow by gravity to supply electrolyte to the tank 4 and spray 17. The settling tank is dumped periodically into 35 the filter 37, the copper powder being washed on the filter, the washing being preferably done with boiled water at a temperature somewhat below 120° F. in order to prevent oxidation. It is then transferred to the vacuum dryer and dried, preferably in accordance with the application of Fitzpatrick et al. mentioned above.

40 The impurities settling out from the anodes are collected by dumping the electrolytic cell tank and allowing the impurities to run into car 37 where they are washed and then dried in a vacuum dryer.

45 All of the copper powder produced as above in accordance with my invention, was removed from the vacuum dryer and found to pass through a 200 mesh screen. The resultant product averaged 99.6% purity. In some instances it was as high as 99.73% pure. The theoretical amount of finely divided copper in pounds that can be produced by 90 hours using a current of about 890 amperes, is equal to 210 pounds. The ampere

efficiency secured by operation of my invention, I have found to be

178  
210 pounds=about 85%.

80

The apparatus is of simple construction. The current density maintained by it varies little, if any, during the operation of the apparatus and consequently the particle size of the resultant copper or other metal is substantially uniform. Since the cathodes are continuously rotating and are being sprayed over their whole surface by the electrolyte, the difficulty of having oxidation at the liquid level of the electrolyte tending to eat away the cathode as in the case of rods used in the old practice, is eliminated. The apparatus and process operate with high efficiency. Furthermore impure anodes may be used thus saving in the expense of these electrodes.

85 As pointed out above other metals than copper which are susceptible to electro-deposition in the manner indicated, may be employed in the apparatus and process described. In addition varying current densities may be employed as required or preferred. It will, of course, be understood that I do not restrict myself to anodes of any particular impurity, but I find it desirable to use a commercial copper as anodes containing approximately a total of .3% of solid impurities as gold, silver, lead, nickel, cobalt, antimony and 90 arsenic.

95 Having thus described my invention with particularly with reference to the preferred method of carrying out the same, it will be obvious to those skilled in the art, after understanding my invention, that various changes and modifications may be made therein without departing from the spirit and scope of my invention, and I aim in the appended claims to cover such changes and modifications as are within the scope of the 100 invention.

105 What is claimed as new and desired to secure by Letters Patent is:—

110 1. A process for making copper powder or the like which comprises, passing a current through an electrolyte bath from an anode to a cathode dissolving the anode in the bath, depositing spongy metal on the cathode scraping off the metal deposit formed on said cathode without 115 passing it through the bath and conveying the deposit away in a non-oxidizing medium.

120 2. A process for making copper powder or the like which comprises, passing a current through an electrolyte bath from a relatively impure anode to a cathode, and removing the deposit from the 125 cathode without passing it through said bath and conveying the deposit away by a stream of electrolyte.

130 3. A process for making copper powder or the like which comprises passing a current through an electrolyte bath from an anode to a cathode while moving the latter, dissolving the anode in the bath, depositing spongy metal on the cathode, scraping off the cathode the metal deposit formed thereon without passing it through 135 the bath, and conveying the deposit away in a non-oxidizing medium.

140 4. A process for making copper powder or the like which comprises passing a current through an electrolyte bath from an anode to a cathode, 145 dissolving the anode in the bath, depositing spongy metal on the cathode, moving the cathode, scraping off the metal deposited thereon without passing it through the bath, and conveying the deposit away in a non-oxidizing medium.

150

5. A process for making copper powder or the like which comprises, passing a current through an electrolyte bath from an impure anode soluble in said electrolyte bath to a moving cathode, and 5 removing the metal deposit formed on said cathode while allowing impurities to settle out in said bath, supplying electrolyte to said bath and withdrawing it therefrom.
6. A process for making copper powder or the like which comprises, passing a current through 10 a heated electrolyte bath from an impure anode soluble in said electrolyte bath to a moving cathode, removing the metal deposit formed on said cathode allowing impurities to settle out in 15 said bath, and continuously supplying heated electrolyte to said bath and withdrawing it therefrom.
7. A process for making copper powder or the like which comprises, passing a current in an electrolyte bath from an anode to a moving 20 cathode, regulating the current density to secure small particles of metal nearly uniform in size on the cathode and scraping off the metal deposit formed on said cathode while protecting the deposit from oxidation by the air, conveying said 25 deposit away to a settling tank, and drying it while substantially preventing oxidation thereof.
8. A process for making copper powder or the like which comprises, passing a current through an electrolyte bath from a relatively impure anode 30 to a cathode, and scraping the deposit from the cathode without passing it through said bath, conveying the deposit away in a stream of electrolyte for protecting the deposit from oxidation by the air and collecting impurities from said 35 anode as said impurities are deposited in said bath and recovering them.
9. A process for making copper powder or the like which comprises, passing a current from spaced relatively impure anode plates to interposed 40 cathodes while rotating the latter in a heated electrolyte bath, regulating the current density to obtain a deposit on the cathodes of nearly uniformly sized particles by adjusting the depth of submersion of said cathodes, scraping 45 off the deposit, and conveying it to a settling tank while protecting it from oxidation by air.
10. A process for making copper powder or the like which comprises, passing a current from spaced relatively impure anode plates to interposed cathode plates while rotating the latter 50 while partially submerged in an electrolyte bath heated to approximately 120° F., regulating the current density to obtain a deposit on the cathodes of nearly uniformly sized particles by adjusting the depth of submersion of said cathodes, scraping 55 off the deposit and conveying it to a settling tank in a non-oxidizing medium, circulating the electrolyte through the bath while maintaining it at approximately 120° F., and dumping the 60
- settling tank periodically into a filter and washing the copper powder thereon.
11. A process for making copper powder which comprises, passing a current from spaced relatively impure copper anode plates to interposed cathode copper discs partially submerged in an electrolyte bath of copper sulphate and sulphuric acid heated to about 120° F. while rotating the cathode discs, regulating the current density to 80 secure small particles of copper of nearly uniform size on the cathodes by adjusting the depth of submersion of the latter in said bath, scraping off the copper deposit and conveying it to a settling tank while protecting it from oxidation by air, circulating the electrolyte through the bath and a receiving tank therefor while maintaining the electrolyte at about 120° F., and dumping the settling tank periodically into a filter and washing the copper powder thereon.
12. A process for making copper powder which comprises, passing a current from spaced relatively impure copper anode plates to rotating cathode copper disks placed between said anodes and submerged edgewise to about one-quarter their depth in an electrolyte bath of copper sulphate and sulphuric acid heated to about 120° F., regulating the current density to secure small particles of copper nearly uniformly sized on the cathodes by adjusting the depth of submersion of said cathodes in said bath, scraping off the copper 105 deposit and washing it into a trough and then into a settling tank and protecting it from oxidation by the air, circulating the electrolyte through the bath, settling tank, and a receiving tank therefor, and past heating coils to keep the liquid 110 in the bath at about 120° F., dumping the settling tank periodically into a filter and washing the copper powder thereon, keeping the said powder submerged in water, then transferring to a dryer and drying, collecting impurities from the anodes 115 as said impurities drop to the bottom of said bath and throwing said impurities on the filter separate from the copper powder and washing and drying the impurities.
13. A process for making copper powder which 120 comprises immersing an impure copper anode in a circulating electrolyte capable of dissolving the anode, rotating a cathode partially immersed in said electrolyte near said anode, passing a current from anode to cathode adapted to deposit spongy 125 copper, depositing copper on said cathode while dissolving the anode, but without depositing impurities on said cathode, scraping off the copper deposit on the cathode and washing it away with a stream of electrolyte to a settling tank, allowing 130 the copper powder to settle and drawing off the electrolyte and returning it to the circulating electrolyte.

JAMES H. LUCAS.

135

65

140

70

145

75

150